

G. MONRATH.  
LINING LAUNDERS.  
APPLICATION FILED JULY 22, 1919.

1,368,960.

Patented Feb. 15, 1921.

Fig. 1,



Fig. 2,



Fig. 4,



Fig. 3,



Inventor  
Gustav Monrath

By his Attorneys

Bennie, Davis, Marin & Edmonds

# UNITED STATES PATENT OFFICE.

GUSTAV MONRATH, OF NEW YORK, N. Y., ASSIGNOR, BY MESNE ASSIGNMENTS, TO THE BARBER ASPHALT PAVING COMPANY, OF PHILADELPHIA, PENNSYLVANIA, A CORPORATION OF WEST VIRGINIA.

## LINING LAUNDERS.

1,368,960.

Specification of Letters Patent. Patented Feb. 15, 1921.

Application filed July 22, 1919. Serial No. 312,475.

To all whom it may concern:

Be it known that I, GUSTAV MONRATH, a citizen of the United States, residing at New York city, in the county of New York, 5 State of New York, have invented certain new and useful Improvements in Lining Launderers; and I do hereby declare the following to be a full, clear, and exact description of the invention, such as will 10 enable others skilled in the art to which it appertains to make and use the same.

This invention relates to the lining of receptacles for liquid, such, for example, as launders, canals, tanks, and the like, and 15 has for its object the provision of an improved lining of asphalt mastic material for the same.

In many metallurgical and chemical plants corrosive or hot liquors are frequently confined in or handled through tanks, launders, canals, and the like, which are most conveniently built of wood or concrete. These receptacles must ordinarily be lined with appropriate material adapted 25 to withstand the corrosive or otherwise deleterious action of the liquors. Asphalt mastic compositions have heretofore been found suitable for the linings of such receptacles, particularly where acid or hot liquors are being handled. Where the 30 receptacles are made of green wood or of concrete which cannot be given time to properly dry, difficulties are encountered in satisfactorily attaching an asphalt mastic lining 35 thereto.

The present invention contemplates an improved lining construction of asphalt mastic material for such receptacles, and in particular for receptacles made of green 40 wood or of concrete that cannot be given time to dry properly. The novel features of the invention which I believe to be patentable are definitely set forth in the appended claims. These features together 45 with the construction of liquid-containing receptacles embodying the same will be understood from the following description taken in conjunction with the accompanying drawings, in which,

50 Figure 1 is a sectional elevation of a wooden launder having an asphalt mastic lining embodying the invention;

Fig. 2 is a perspective view partly in sec-

tion of an asphalt mastic block or slab of the lining of the launder;

55

Fig. 3 is a sectional view of a concrete tank having an asphalt mastic lining embodying the invention; and

Fig. 4 is a perspective view partly in section illustrating the mode of making the 60 asphalt mastic blocks or slabs of the lining of the tank.

The launder of Fig. 1 has an outer structure or frame 5 of wood, such, for example, as green or imperfectly seasoned wood. In 65 accordance with the present invention, the wooden frame 5 is provided with an acid proof lining made up of blocks or slabs 6 of asphalt mastic material. The slabs 6 are of a size suitable for the work in hand and 70 are from  $\frac{1}{2}$  inch to  $1\frac{1}{2}$  inches in thickness. A reinforcement 7 of expanded metal, or other suitable reinforcing agent, is embedded in each slab. The slabs may be made in any appropriate manner, as, for example, 75 by pouring the asphalt mastic material, heated to a sufficiently high temperature to secure the desired fluidity for casting, into a mold or form of suitable dimensions.

The asphalt mastic slabs 7 are attached 80 and secured to the sides of the wooden frame 5 by screws 8 countersunk in the slabs with their heads covered with hot mastic. In Fig. 1 of the drawings I have indicated the slabs 7 similarly secured to the 85 bottom of the wooden frame 5, but this is not necessary, since the bottom lining will remain in place without the screws 8. The joints between adjacent slabs and between the slabs and the sides and the bottom of 90 the wooden frame 5 are cemented with hot mastic.

In Fig. 3 of the drawings, I have shown a concrete tank 10 lined with asphalt mastic blocks or slabs 11. The slabs 11 have a 95 back 12 of clean crushed stone partly embedded in the asphalt mastic. In Fig. 4 of the drawings I have indicated a convenient way of making the slabs 11. The mold or form 15, of suitable dimensions to produce a slab of the desired size, is placed horizontally on the ground. The bottom of the form 15 is covered with a thin layer of crushed stone, of about  $\frac{1}{8}$  inch mesh. The asphalt mastic material, heated to a sufficiently high temperature to secure the de- 100 105

sired fluidity for casting, is then poured over the stones flush with the top of the form. A reinforcement 13 of expanded metal, or other suitable material, is preferably embedded in the slab in any convenient manner. When the slab cools off it will have a back of clean crushed stones partly embedded in the asphalt mastic material.

In placing the slabs 11 on the sides of 10 the tank 10, a thin coat of cement mortar 14 is spread over the back of the slabs and the slabs are pressed against the concrete. The joints between the slabs of the side wall 15 lining of the tank are cemented with hot mastic. Similarly, the joints between adjacent slabs and between the slabs and the bottom of the concrete tank are cemented with hot mastic.

From the foregoing description it will be 20 evident that the asphalt mastic lining, made up of blocks or slabs, is securely attached to the side walls of the receptacle. The back of clean crushed stone partly embedded in the mastic provides a surface of suitable 25 character for cementing the asphalt mastic slab to the concrete by means of a cement mortar. As previously mentioned, the attaching means of the invention for securing the asphalt mastic slabs to the receptacle 30 have been found satisfactory for receptacles made of green wood or concrete that can-

not be given time to properly dry, thus enabling the use of green wood and concrete under conditions which have heretofore been considered not conducive or satisfactory for the proper lining thereof with asphalt mastic material. The reinforcing member embedded in the slabs increases the durability of the lining, and prevents bulging and other distortion of the asphalt 40 mastic slabs as the result of softening from the effects of hot liquors, or as the result of other causes.

I claim:

1. A lining slab for liquid receptacles 45 comprising asphalt mastic and a backing of crushed stone partly embedded in the mastic.

2. A lining slab for liquid receptacles comprising asphalt mastic material, a reinforcing element therein and a backing of crushed stone partly embedded in the mastic.

3. In a concrete receptacle for liquids, a lining made up of slabs of asphalt mastic material having a back of crushed stone 55 partly embedded in the mastic material, and a coating of cement mortar for cementing the backs of the slabs to the side walls of the concrete receptacle; substantially as described.

In testimony whereof I affix my signature.  
GUSTAV MONRATH.